

# UNITED STATES PATENT OFFICE.

WALTER COSBY, OF SAN FRANCISCO, CALIFORNIA.

## EXPLOSIVE CONTAINING NITROGLYCERIN.

1,205,516.

Specification of Letters Patent. Patented Nov. 21, 1916.

No Drawing.

Application filed July 8, 1916. Serial No. 108,220.

To all whom it may concern:

Be it known that I, WALTER COSBY, a citizen of the United States, and resident of San Francisco, in the county of San Francisco and State of California, have invented certain new and useful Improvements in Explosives Containing Nitroglycerin, of which the following is a specification.

The present invention relates to explosives and more particularly to new and useful improvements in desensitizing compounds for nitro-glycerin and the like.

The primary object of my invention is to provide a new and improved composition of matter adapted for incorporation with nitro-glycerin whereby to render the same less susceptible to explosion due to accidental shock or the like.

Another object of my invention is to provide a compound of the class described to be combined with nitro-glycerin whereby to render the same more safe for handling and shipping by desensitizing nitro-glycerin without destroying any of the explosive qualities of the same.

Other objects and advantages to be derived from my improved desensitizing compound will appear from the following detail description and the claims.

It is, of course, well known to those skilled in the art that the globular normal condition of nitro-glycerin accounts for the sensitiveness of the nitro-glycerin and its liability of accidental ignition.

Referring specifically to the compound and its constituent parts I combine carbon tetrachlorid ( $CCl_4$ ) and carbon dichlorid ( $C_2Cl_4$ ), the former being known as tetrachlormethane and the latter being known as tetrachlorethene. The ingredients mentioned may be either collectively or independently combined with nitro-glycerin.

The best form of my new explosive compound as determined by experiment, results from adding 20 per cent. tetrachlormethane to 80 per cent. nitro-glycerin, or the same proportions may be used by substituting tetrachlorethene for the tetrachlormethane. I have also found that a compound equally efficient as the above may be prepared by

adding 20 per cent. tetrachlormethane and tetrachlorethene in relative proportions and 80 per cent. nitro-glycerin.

The purposes of the tetrachlormethane and tetrachlorethene are to destroy the globular condition in which sensitive nitro-glycerin usually is found, also preventing flame propagation.

I have discovered by actual test that when nitro-glycerin is combined with the ingredients of my invention accidental explosion is practically impossible. This will be evident from the fact that by destroying the globular condition of normal nitro-glycerin I remove the danger of accidental explosion. It will, therefore, be seen that in the provision of my improved desensitizing compound I afford means for rendering more safe the handling of nitro-glycerin and similar explosives without the reduction of efficiency of the explosive.

From the above description it is thought that a clear and comprehensive understanding of the constituent parts and the uses of my improved compound may be had, and while I have described a specific combination of elements it is to be understood that I do not limit myself to the proportions set forth but reserve the right to make changes therein such as do not depart from the spirit and scope of the invention as claimed.

Having thus fully described my invention, what I claim as new and desire to secure by Letters Patent, is:

1. An explosive compound consisting of nitro-glycerin and tetrachlorethene in the manner and proportions set forth.
2. An explosive compound consisting of nitro-glycerin, 80 per cent. and tetrachlorethene, 20 per cent.
3. An explosive compound consisting of nitro-glycerin, tetrachlormethane and tetrachlorethene, all combined in the manner and proportions set forth.
4. An explosive compound consisting of nitro-glycerin, 80 per cent., tetrachlormethane and tetrachlorethene; 20 per cent.

In testimony whereof, I affix my signature hereto.

WALTER COSBY.